

No. 846,297.

PATENTED MAR. 5, 1907.

W. M. FULTON.

PROCESS OF MAKING COLLAPSIBLE AND EXPANSIBLE VESSELS.

APPLICATION FILED NOV. 2, 1904.

Fig. 1.



Fig. 2.



Fig. 3.



Fig. 4.



Inventor

Weslon M. Fulton,

By

Witnesses

Mrs. Weston

Maurice R. Thompson.

Mauro. Cameron, Lewis Braxton,  
Attorneys.

# UNITED STATES PATENT OFFICE.

WESTON M. FULTON, OF KNOXVILLE, TENNESSEE, ASSIGNOR TO THE FULTON COMPANY, OF KNOXVILLE, TENNESSEE, A CORPORATION OF MAINE.

## PROCESS OF MAKING COLLAPSIBLE AND EXPANSIBLE VESSELS.

No. 846,297.

Specification of Letters Patent.

Patented March 5, 1907.

Original application filed July 19, 1904, Serial No. 217,286. Divided and this application filed November 2, 1904. Serial No. 281,120.

*To all whom it may concern:*

Be it known that I, WESTON M. FULTON, of Knoxville, Tennessee, have invented a new and useful Process of Making Collapsible and Expansible Vessels, which invention is fully set forth in the following specification.

This invention relates to a process of treating sheet metal, and has for its object the production of walls for corrugated vessels which shall have substantially uniform density and great flexibility and durability.

In a previous application for Letters Patent, Serial No. 213,864, filed June 23, 1904, I have described a process for electrically welding sheet steel. Collapsible vessels of sheet-steel having seams electrically welded have great durability and flexibility; but it is desirable at times to have the flexible wall of a collapsible and expansible vessel made of metals not readily weldable, such as copper and brass, and which resist the oxidizing action of air and moisture. Such vessels are especially useful when the vessel is to be employed, for example, as the expansible portion of a steam-gage or as the thermosensitive portion of devices for gaging the temperatures of liquids. In devices of this character steel readily corrodes and is not serviceable even when protected by metal coatings of tin, zinc, or nickel, because the best of such coatings are porous and crack in use, exposing the iron to oxidation and rusting.

In my application, Serial No. 217,286, filed July 19, 1904, I have described corrugated sheet-metal walls for use in collapsible and expansible vessels and the process of making the same and have claimed the article therein. In the present application, which is a division of application Serial No. 217,286, I have described and claimed the process of making such articles of manufacture. It is desirable to use in flexible vessels of this kind a metal or alloy that will not readily corrode, such as copper or brass. In making the walls of collapsible vessels out of copper or brass it has been found that the seams readily give way to bending strains and break. Therefore seamless drawn tubing is preferable for constructing such vessels; but even seamless drawn tubing soon develops weakness at the bends in the corrugations, which unfit it for use in constructing the walls of corrugated collapsible vessels. In the manufacture of seamless tubing one of the common methods

in use is to draw the tube between a mandrel and die. This operation results in condensing and hardening the outside layers of the metal wall, leaving the inner portion of the wall more or less unaffected in these respects. The dense outer layers possess quite different molecular structure from the inner layer in their physical qualities, such as hardness, brittleness, expansion, and contraction under influence of heat, and also in elasticity. In the case of brass tubing made in this way the coefficient of expansion of the dense layers differs so widely from that of the inner layer that the ordinary changes in atmospheric temperatures causes the tube to crack. Although annealing reduces this difference in molecular structure between the layers and prevents cracking for ordinary purposes, yet such annealing fails to render the drawn tubing serviceable for making the walls of flexible corrugated collapsible vessels which are to withstand repeated expansion and compression.

To better understand this invention and how the difficulties above noted have been overcome, reference is had to the accompanying illustrations, in which—

Figure 1 shows a tube drawn from a cast ingot in the usual way. Fig. 2 is a longitudinal section of the same. Fig. 3 is the tube of Fig. 1 corrugated, and Fig. 4 shows the tube on a mandrel.

1 indicates a die-drawn seamless tube of metal, such as brass, having its end 2 highly magnified for the sake of illustrating the molecular condition of the wall.

3 and 4 are the inner and outer portions of the tube, which have been compressed and hardened by contact of the mandrel and die, respectively, in the course of its manufacture, and 5 is the intermediate layer farthest removed from the compressing action during drawing. The relative density of the several layers is also indicated by the dotted shading. It will thus be seen that the wall of a die-drawn tube is not of homogeneous structure in passing through the wall from one side to the other, but is composed of layers more or less clearly defined which possess different degrees of hardness and different coefficients of expansion. By reason of this lack of uniform constitution deleterious effects result and become serious when such tubing is made into a corrugated collapsible vessel.

In Fig. 3 is illustrated the walls of a corrugated vessel shown in section. 6 designates a single corrugation. If the wall is collapsed, the outer layer 4 will be compressed, while 5 the layer 3 will be drawn out. The middle layer 5, which is relatively neutral, will serve to intensify the strain on layers 3 and 4 by virtue of the fact that it separates them from each other. When the wall is expanded, the 10 reverse action takes place. These repeated strains acting upon these several layers of different molecular structure alternately in opposite directions causes an ultimate separation of the layers and cracks in the outer 15 layers which, once formed in the surface, extend through the wall, rendering it useless.

It is therefore the object of this invention to produce sheet-metal walls for collapsible and expansible vessels which are free from 20 the objections noted and which shall be of more uniform density throughout the thickness of the wall and be flexible and durable. To accomplish these objects, one or more of the non-homogeneous layers composing the 25 sheet of metal is removed, preferably by the mechanical action of a tool; but the removal of the layer or layers may be effected by means of a suitable solvent or by electrolysis.

To illustrate one method of carrying out 30 the invention, a seamless tube is formed, preferably of brass, by any of the well-known methods, such as by drawing a tube from a cast ingot. This tube is then chucked in a lathe, and by means of a boring bar and tool the inner 35 condensed layer is removed. The tube is then placed on a mandrel 7, (shown in Fig. 4,) having its surface trued and of just sufficient diameter to fit closely the inside of the tube 1. This mandrel, with its tube upon it, 40 is then chucked in a lathe and the outer surface removed. The remaining tube is then corrugated deeply, as indicated in Fig. 3, and there results a flexible elastic corrugated wall which may be elongated and compressed 45 and which will withstand repeated strains without danger of cracking.

In illustrating this invention a seamless die-drawn metal tube has been taken and the two condensed surfaces removed; but the 50 method is equally applicable to sheet metal not in the form of a tube, such as sheet metal which has been rolled and has its outer layers thereby hardened and before or after shaping it into its final configuration. The tube may

not be die-drawn, but may be made from sheet metal, preferably sheet-brass, by bending the sheet into cylindrical form, butting the edges, and brazing. The tube is then treated in a similar manner as one die-drawn and then corrugated to form the flexible elastic wall.

Although excellent results are obtained by removing both surfaces of the sheet metal, yet only one may be removed and the advantages of the process be apparent in the result. 65 It is found, however, that by removing fifty percent. to eighty per cent. of the thickness of the wall the best results are obtained, and I preferably use seamless drawn tubing; but seamless brazed tubing may be used. The 70 removal of the layers is performed in the same manner as with drawn tubing. This method greatly improves the walls of collapsible vessels made of metals not usually weldable, imparting to the wall great durability 75 and flexibility. Brass and copper sheet metal thus treated and corrugated are greatly improved and better adapted for use in constructing the walls of corrugated expansible and collapsible vessels.

What is claimed is—

1. A process of making substantially homogeneous flexible corrugated-metal walls for expansible and collapsible vessels from rolled or drawn sheet metal having its outer 85 surfaces more condensed than the interior portion, consisting in removing said condensed surfaces and corrugating the substantially homogeneous remaining portion of said sheet.

2. A process of making substantially homogeneous flexible corrugated-metal walls for expansible and collapsible vessels from metal tubing having surfaces more condensed than the interior portions of the wall 95 of the tubing, said process consisting in removing from said tubing the condensed surfaces of the wall and corrugating the substantially homogeneous remaining portion of the wall of the tubing.

In testimony whereof I have signed this specification in the presence of two subscribing witnesses.

WESTON M. FULTON.

Witnesses:

JOHN S. BROWN,  
W. W. BERRY.